

July 16, 1935.

J. L. McCLELLAN

2,008,141

INSULATING OR "FISH" PAPER AND METHOD OF MAKING

Filed March 24, 1931

Fig. 1



Fig. 2



INVENTOR  
JAMES L MC CLELLAN  
by Robert, Cushman & Woodbury  
ATTYS

## UNITED STATES PATENT OFFICE

2,008,141

INSULATING OR "FISH" PAPER AND  
METHOD OF MAKINGJames L. McClellan, Littleton, Mass., assignor to  
Hollingsworth & Vose Company, Boston, Mass.,  
a corporation of Massachusetts

Application March 24, 1931, Serial No. 524,851

15 Claims. (Cl. 151—34)

This invention relates to papers which are especially suitable for electrical insulating purposes and the like and to a method of making the same.

- 5 Papers heretofore made for use in electrical insulations have been prepared with respect to the improvement of their electrical resistance or dielectric strength but such improvements have usually been effected at the expense of their 10 physical properties, such as mechanical strength, toughness, flexibility, etc. Consequently, the insulating or "fish" papers, so-called, which are now available, are either of low dielectric strength or of a weak, brittle, mechanical structure.
- 15 It is therefore an object of the present invention to provide an electrical insulating paper which shall have both a high dielectric or insulating value and also a high degree of mechanical strength or toughness, and which shall be 20 adapted to resist the strains of folding and shaping as well as the wear incident to its subsequent use, without interruption of its structural continuity. Other objects will appear from the following disclosure.
- 25 It is found as a part of this invention that fibers,—typically those derived from long fiber leaves namely the true hemp, such as manila and sisal hemp, in contradistinction to jute or bast fibers, and cotton, as well as straw and the like,—are not only strong and tough but may be 30 formed into sheets of paper and so treated that they shall preserve substantially the original strength of the individual fibers and also acquire a high dielectric strength or resistance to the 35 passage of the electric current.

The fibers which are thus suitable belong generically to the musaceæ or banana family and include more specifically the fibers which are known as manila and sisal hemp. These fibers 40 are available in the form of the freshly prepared material but are more commonly obtained as old rope which has been made from these fibers. Common hemp and jute, however, which are bast fibers, are not suitable.

45 The process of the present invention includes, generally, the reduction of the fiber or rope to short lengths (e. g., two inches, more or less) which are then beaten out to separate the fibers and may be subjected to an alkaline cooking 50 treatment in a digester and under pressure for a sufficient time to produce a pulp. This pulp may then be formed into an absorbent sheet of paper in any of the customary ways for making manila fiber papers. Preferably, however, the 55 sheet is so made (by adjustments of the stock and

control of the paper-making operation, in ways well known by those skilled in the art) that it presents a relatively open, absorbent structure. Thus, for purposes of the present invention, the open structure of the sheet is so controlled that subsequent impregnation, even by active reagents which tend to swell the cellulosic compounds of the paper and thus close the interstices, may be effected to the desired degree throughout the sheet. Other things being equal, it may be desirable to employ a relatively more porous sheet when thick, and a less porous sheet when thin.

In any event, the paper is especially characterized by a tough fibrous structure in which the original fibers have not been materially weakened and compose a considerable proportion of the stock. In some instances, cellulosic materials, which are subject to parchmentizing, may be added to provide an additional matrix or bonding material for the tough fibers, but the amounts of such materials should be limited in order to avoid loss of strength in the finished product.

It is further found that the paper sheet thus obtained may be subjected to a parchmentizing treatment, as by passing the same through a parchmentizing solution of sulfuric acid, zinc chloride, or the like,—preferably at such temperature and for such time, in connection with the weight or thickness of the sheet, as to permit thorough penetration of the sheet by the parchmentizing solution,—the rate and degree of the parchmentizing effect being controlled in part by the concentration of the solution used. The treated sheet is then washed free from the parchmentizing reagents, dried, and calendered to provide the desired thickness, density and finish, according to known methods of the paper-making art.

A typical instance of carrying out the invention will be described with reference to the accompanying drawing, in which

Fig. 1 is a diagrammatic side elevation of suitable apparatus therefor; and

Fig. 2 illustrates drying and calendering equipment.

For example, paper, which has been prepared from sisal or manila hemp fibers, or both, as above described and which is of a relatively open structure, is shown in the form of one or more 50 rolls,—e. g., as indicated at 1, 2, 3 and 4, respectively. These sheets may also contain additions of more parchmentizable material, if desired, such as cotton or other forms of cellulosic material, which has been incorporated with the 55

sisal or manila fiber in the beater. All four sheets may be composed of sisal or manila fibers, for maximum strength in the finished sheet or one or more sheets may be composed of alpha cellulose or cotton fiber, if desired, for special purposes, such as to provide an intervening layer or matrix of readily parchmentized cellulose. Other numbers and arrangements of such sheets may also be provided for and integrated together, in like manner.

The sheets are drawn, in parallel, into and through a tank 5 containing a parchmentizing solution,—e. g., a 70° Baumé solution  $ZnCl_2$  in water, which is maintained at about 100° F. The degree of penetration and parchmentizing effect of the solution upon the sheet may also be controlled by the rate at which the sheets travel and the length of the tank. It may be still further regulated by passing each sheet through a separate tank (not shown) having correspondingly prepared and regulated parchmentizing solutions therein to effect the desired parchmentizing action upon each sheet severally.

In passing through the tank (or tanks) 5 the sheets 1, 2, 3 and 4, are guided by rolls 6, 7, 8, 9 and 11, 12, 13, 14,—and upon leaving the parchmentizing solution they are associated in intimate face contact. The composite sheet is then passed over a heated calender roll 15 (preferably heated, e. g., to 100° F.) and then between the upper roll 15 and the lower calender roll 16, which may also be heated, (e. g., to 120° F.) In thus passing between the calender rolls, the sheets are integrated into a single sheet of substantially uniform, continuous structure. The thus integrated sheet 17 may be passed over spaced guide rolls 18, 19, 21, while they are freely exposed to the air, thus permitting the parchmentizing action to become more completely effective throughout the sheet. By suitably spacing the rolls 18, 19 and 21, the length of time, etc., of such "aerating treatment" may be adjusted to the desired degree.

The sheet is then subjected to a thorough washing treatment, which is effected by passing through a long series of washing tanks 22, 22, or other appropriate apparatus. As shown, the sheet is conveyed, alternately over upper rollers 23, which may be connected to a suitable source 50 of power (not shown) to drive the same, and under lower rollers 24, which are mounted near the bottom of the successive tanks 22 of the series. These rollers 24 are customarily mounted in frames (not shown) which may be raised from 55 and lowered into the tanks, as desired, in order to thread and rethread the paper sheet therethrough. In operation, the tanks are periodically emptied,—the contents of the first tank being withdrawn and the waste water from each 60 succeeding tank being advanced, the last tank of the series being filled with fresh water.

At the end of the series of washing tanks, the washed sheet may be passed over a series of drying drums 26, 27, and thence through calendar 65 rolls 28, if desired, and finally wound up in a roll, 29, which constitutes the finished product.

It is found that the parchmentizing treatment, while substantially ineffective to soften or weaken the hard fibers of the type indicated, is nevertheless sufficiently reactive upon a portion of the paper stock to provide a bond between the tough fibers and also to fill the interstices, thus forming a relatively dense, impervious sheet. Moreover, this interfibrile parchmentized material or matrix is characterized by high dielectric

strength. At the same time, it is relatively soft and flexible, so that it preserves its continuity and bonding adhesion to the fibers in spite of repeated and drastic folding.

If for any reason, the particular fiber employed does not contain a sufficient amount of such bonding material or if it is not rendered available by the desired parchmentizing treatment, additions of cellulosic materials which are especially susceptible to the parchmentizing treatment (preferably cotton pulp) may be made advantageously as pointed out above.

In either case, the strong and tough, undegenerated fibers form an interlacing network throughout the paper sheet, imparting both strength and toughness thereto which permit the finished sheet to be sharply bent or folded, without rupture on the stretched side of the fold nor buckling or delamination in the compressed side of the fold. Consequently the continuity and structure of the sheet is preserved and its dielectric strength as well as its mechanical strength remains unimpaired. That the paper has an intrinsically high value in respect of these properties, as compared with "fish" paper heretofore produced is indicated by the data obtained in tests upon paper made as above described in which it was found that:

(1) The dielectric strength (volts per mm. of thickness) is more than doubled.

(2) The tearing strength (grams per millimeter of thickness) is approximately doubled; and

(3) The folding strength (number of folds before rupture) is greatly improved.

Not only is the paper thus prepared stronger than the unparchmentized sheet, but it is more resistant to abrasion and will not delaminate or separate into the layers of which it is initially composed. If split, by cutting at the edge for example, and torn apart, it not only presents high resistance to such separation but does not tear continuously in this plane. On the contrary the torn section tapers off to the outer surface of the sheet, and no evidence of an irregular or delaminated structure is observable.

Another feature of the product is a characteristic increase of tensile strength upon wetting of the sheet with water, which continues with increasing amounts of water up to such degree of saturation as it is capable of.

While the resulting product is thus particularly advantageous for use as an insulating paper, it is clear that its properties of strength, toughness, etc., and the preservation of these properties in spite of repeated folding or wear, make it especially applicable for many other applications and uses in which its dielectric properties may not be of importance.

Other modifications and adaptations of the method and applications of the product are therefore contemplated and are to be considered as included by the following claims.

I claim:

1. Method of treating paper, comprising as a step subjecting paper containing true hemp fibers to a parchmentizing treatment.

2. Method of making paper, comprising as steps preparing an absorbent sheet of paper from sisal and/or manila hemp fiber and subjecting the same to a parchmentizing treatment.

3. Method of treating paper, comprising as a step subjecting paper containing sisal and/or manila hemp fibers and additional cellulosic material, to a parchmentizing treatment.

4. Method of making paper, comprising as steps

- preparing an absorbent sheet of paper, containing true hemp fibers and a cellulosic material, and subjecting the same to a parchmentizing treatment.
5. Paper, consisting substantially of true hemp fibers and characterized by being parchmentized.
6. Paper, consisting substantially of sisal fibers and characterized by being parchmentized.
7. Paper, consisting substantially of manila fibers and characterized by being parchmentized.
10. Paper, containing true hemp fibers and other cellulosic material, and characterized by being parchmentized.
8. Paper, containing true hemp fibers and other cellulosic material, and characterized by being parchmentized.
15. Paper, containing sisal fibers and other cellulosic material, and characterized by being parchmentized.
10. Paper, containing manila fibers and other cellulosic material, and characterized by being parchmentized.
11. Paper, characterized by containing true hemp fibers and a bonding matrix of parchmentized cellulosic material.
12. Paper, containing true hemp fibers and a layer of cellulosic material, the whole characterized by being parchmentized.
13. Paper, characterized by containing true hemp fibers and a layer of other cellulosic material, said cellulosic layer being parchmentized.
14. Paper characterized by high dielectric capacity and flexibility, and containing sisal or manila hemp fibers and a bonding matrix of parchmentized cellulosic material.
15. Paper characterized by high dielectric capacity and flexibility, and containing sisal or manila hemp fibers and a layer of parchmentized cellulosic material integrated therewith.

JAMES L. McCLELLAN.